

# UNITED STATES PATENT OFFICE.

HUGO COHN, OF MOYS, GERMANY.

## MANUFACTURE OF PAPER OR PASTEBOARD.

SPECIFICATION forming part of Letters Patent No. 655,850, dated August 14, 1900.

Application filed March 28, 1899. Serial No. 710,817. (No specimens.)

*To all whom it may concern:*

Be it known that I, HUGO COHN, manufacturer, a subject of the Emperor of Germany, and a resident of Moys, in the Empire of Germany, have invented certain new and useful Improvements in the Manufacture of Paper or Pasteboard, of which the following is a specification.

This invention has for its object the manufacture of paper or pasteboard capable of receiving impressions and applicable for use in metal-casting and in the production of stereotype-matrices, embossed wall-papers, and the like by so changing the structure of suitable raw materials—such, for instance, as cellulose, rags, residues of material, and paper scraps or residues from the manufacture of paper—by treatment with caustic-soda lye that the fibers are separated and curled up. By this curling of the fibers hollow spaces are formed in the paper or pasteboard prepared therefrom, which make the product looser or more porous and capable of receiving impressions. If the surface of the paper or pasteboard thus produced be given a suitable coating of china-clay, French chalk, talc, or the like, it is rendered non-susceptible to heat, whereby the paper or pasteboard is adapted for use as a matrix in casting stereotype-plates. The making of such paper and pasteboard is preferably carried out most cheaply from paper scraps or residues free from wood.

In carrying the invention into effect such paper scraps or materials are conveyed into a tank provided with a kneading and mixing apparatus after the tank has been filled with a caustic-soda solution of 9° Baumé and it is heated to about 100° centigrade. The raw material is disintegrated in about two hours and the lye is pumped off, which process is facilitated if the tank be provided with a double bottom, the upper one of which is perforated in the form of a sieve. The pumped-off lye can always be again utilized for disintegrating fresh raw material. The half-stuff thus obtained is washed with hot water and conveyed into a rag-engine, which grinds it into fully-prepared material, after which it is neutralized by the addition of hydrochloric acid. In order to make paper and pasteboard from the material thus treated, a Fourdrinier

machine with an upper wire is employed which must have no press-roll and no suction device, in order that the fibers may remain in their loose crinkled or curled position. By this means the paper or pasteboard reaches the drying-cylinder with about ninety degrees of water, and gauze must be used instead of the usual drying-felt to allow this large amount of moisture to better escape from the paper and pasteboard. The resulting product is a soft open porous paper or pasteboard, according to whether it has been allowed to run onto the Fourdrinier machine in a thick or thin layer and which is adapted to receive an impression under the slightest pressure and which does not allow the impression to again disappear. In other words, the impression is permanent.

If the paper or pasteboard is to be used as a matrix and rendered resistant to molten metal, the upper surface is coated, while the paper or pasteboard is traveling over the drying-cylinder, by means of a rotary brush-roller with a finish or paste formed as follows: ten kilograms of china-clay and ten kilograms of talc are mixed in one hundred liters of water, and to this are added one hundred liters of an emulsion produced by boiling three kilograms of quince-seeds (*Semen cydoniae*) in two hundred liters of water. This white finish is conveyed into a vessel fitted with a stirring apparatus, from which it flows into a box in which a brush-roller revolves, over which the paper or pasteboard band is conveyed.

If the paper or pasteboard is to be employed for forming relief or embossed wall-papers, it is passed between the rollers of a roller-press the upper cylinder of which has a pattern deeply engraved. By this means the pattern is embossed on the paper or pasteboard, while the flat spaces between the pattern are compressed, and thereby become thinner and harder. If the engraved roller be brought in contact with colored rollers, any desired color or bronzing or shade may be imparted to it, and by means of a suitable covering layer an imitation of leather wall-hanging may be produced.

If it be desired to render the wall-hangings or wall-paper resistant to moist walls, the rear side is allowed to travel over a rotating brush-

roller, which conveys onto it a shellac solution.

If the paper or pasteboard is to be made of cellulose, the process is precisely the same as the one already described in which waste paper is used; but if it is to be made from rags or fragments of fabrics they are first cut and the dust beaten out and then washed and ground in a rag-cylinder to half-stuff, which are then brought into the drip-box, the water pressed out and afterward conveyed into the lye-tank, and then further treated in the manner hereinbefore described.

Having thus described my invention, the following is what I claim as new therein and desire to secure by Letters Patent:

1. The process for the manufacture of paper or pasteboard, which consists in treating vegetable fibers with warm caustic lye of 9° Baumé at a temperature of about 100° centigrade, for about two hours in order to ruffle or curl the fibers, washing the fibrous material in hot water, subjecting the mass to the usual beating until it becomes an integral mixture, neutralizing the pulp with muriatic acid spreading it in a film without pressure or suction for the purpose of laying the

felted fiber without compressing it; substantially as described.

2. The process for the manufacture of paper or pasteboard, which consists in treating vegetable fibers with warm caustic lye of 9° Baumé at a temperature of about 100° centigrade, for about two hours in order to ruffle or curl the fibers, washing the fibrous material in hot water, subjecting the mass to the usual beating until it becomes an integral mixture, neutralizing the pulp with muriatic acid spreading it in a film without pressure or suction, for the purpose of laying the felted fiber without compressing it, and covering the pulp with a layer or coating consisting of a mixture of about one hundred liters of water, ten kilograms of china-clay and ten kilograms of talcum, and about one hundred liters of water having one and one-half kilograms of quince-seeds boiled therein; substantially as described.

In witness whereof I have hereunto set my hand in presence of two witnesses.

HUGO COHN.

Witnesses:

HENRY HASPER,

WOLDEMAR HAUPT.